

# United States Patent Office.

CYRUS B. MORSE, OF RHINEBECK, NEW YORK.

*Letters Patent No. 97,953, dated December 14, 1869; antedated December 8, 1869.*

## IMPROVEMENT IN CAST-STEEL TUBE OR INGOT.

The Schedule referred to in these Letters Patent and making part of the same.

*To all whom it may concern:*

Be it known that I, CYRUS B. MORSE, of Rhinebeck, in the county of Dutchess, and State of New York, have invented a new and improved Cast-Steel Ingot; and I do hereby declare that the following is a full, clear, and exact description of the mode of producing the same:

The object of this invention is to produce hollow ingots or tubes of highly-carbonized cast-steel, which will possess all the qualities of the best tool or cutlery-steel, and admit of being drawn under the hammer or rolling-mill to the required thickness, diameter, and length, for conversion into a variety of useful articles which have hitherto been made of iron or low steel, by punching or welding, such, for instance, as steam-pipes, gun-barrels, boiler-flues, tubular flues, tubular shafting, hollow axles, axle-boxes, spindles, locomotive, marine, or other flues, and rings for spinning-frames and other purposes.

The difficulty hitherto experienced in attempts at the production of highly-carbonized steel ingots or tubes, by casting them in moulds, is chiefly owing to the extreme brittleness and intractability of steel when it is charged with carbon above, say, one per centum, and also the porosity and imperfections of the steel after it is moulded.

These difficulties I have overcome, by a process or treatment which is exceedingly simple and equally effective.

I will commence, by stating the several ingredients entering into the composition of the steel which I prefer to use, and their relative proportions.

For a pot of steel weighing fifty pounds, I take about thirty pounds of Peru or Swedish iron, twenty pounds of scrap-steel, five ounces of charcoal-powder, six ounces of refined manganese, and three ounces of rock-salt.

These substances are melted together until the mass attains a very high degree of heat, and becomes what is technically known as dead steel. It is then skinned, to remove these floating impurities, and allowed to stand until it is ready for pouring.

After conversion, the steel, which is carbonized to a high degree, say one per centum, is poured from the melting-pot into a cylindric mould, of suitable dimensions, containing a core in its centre, which will produce a tube or hollow ingot.

The mould may be made in the usual manner for casting cast-steel ingots, with these important differences, to wit:

Near the bottom of the mould, where the two halves or sections join, small holes or conduits are made through its walls, which are designed for allowing a free escape of air from the bottom of the mould-chamber during the filling thereof with steel, and thus prevent imperfections in the castings, danger from explosion, or expulsion of the liquid metal from the mould, which would be liable to occur if the air-vents were not made, as stated.

The core, which is arranged centrally in the mould, may be made of a cylindrical bar of cast-steel; or it may be made of a mixture of sand and flour, with a hole through its centre, for allowing the upward and downward escape of air and gas from the mould-chamber while pouring in the steel.

If the core is made of metal, the ingot, in cooling, will contract very firmly around it, and may be removed by heating and expanding by hammering; and if the core is made of sand, it can be readily broken up and cleared out of the ingot, after the latter has cooled.

I attribute my success in the production of highly-carbonized steel castings, chiefly to the free escape of air and gas from the mould during the operation of pouring the metal therein. In the case of the hollow sand core, the air and gas will pass off freely through it, and may be observed, in the form of blue flame, issuing from each end of the core; and in the case of the metal core, the air escapes from the mould, near its base.

Hollow ingots thus produced will be highly carbonized, and when properly heated, may be drawn, by hammering or rolling them, and a great variety of useful articles may be produced from them, without weld or seam.

Having described my invention,

What I claim as new, and desire to secure by Letters Patent, is—

As a new article of manufacture, a cast-steel tube, which is produced substantially as described.

C. B. MORSE.

Witnesses:

JULIUS HIRSCH,

R. T. CAMPBELL.